

# United States Patent

[19]

Yamamoto et al.

[11] 3,870,525

[45] Mar. 11, 1975

[54] **PROCESS FOR PRODUCING  
PHOTOGRAPHIC FILM HAVING A  
MAGNETIZABLE LAYER THEREON AND  
SUCH A PHOTOGRAPHIC FILM**

[75] Inventors: **Nobuo Yamamoto; Hideo  
Kawaguchi; Katsuhiro Furukawa,**  
all of Minami Ashigara, Japan

[73] Assignee: **Fuji Photo Film Co., Ltd.,**  
Kanagawa, Japan

[22] Filed: **Apr. 24, 1973**

[21] Appl. No.: **354,055**

[30] **Foreign Application Priority Data**  
Apr. 12, 1972 Japan ..... 47-41123

[52] **U.S. Cl.** ..... 96/39, 96/84 R, 117/235,  
117/239

[51] **Int. Cl.** ..... G03c 5/14, G03c 1/84, C22c 39/00

[58] **Field of Search** ..... 96/84 R, 4, 39; 117/235,  
117/239

## [56] References Cited

### UNITED STATES PATENTS

3,649,541 3/1972 Ingersoll ..... 117/235

3,689,317 9/1972 Akashi et al. .... 117/235  
3,704,167 11/1972 Yamamoto et al. .... 117/239  
3,773,539 11/1973 Sato et al. .... 96/84 R

## FOREIGN PATENTS OR APPLICATIONS

1,147,399 4/1963 Germany ..... 117/235

*Primary Examiner*—Mary F. Kelley  
*Attorney, Agent, or Firm*—Sughrue, Rothwell, Mion,  
Zinn & Macpeak

## [57] ABSTRACT

A process for producing a photographic film having thereon a magnetic recording layer by applying a dispersion of a magnetic substance to an antihalation layer of a light-sensitive film for cinema, where the dispersion contains a compound or compounds, having at least two or more isocyanato groups or thioisocyanato groups or the anti-halation layer is previously processed with a solution containing the compound. A photographic film where either the magnetic layer contains, or the antihalation layer has been processed with, such a compound or compounds.

**21 Claims, No Drawings**

**PROCESS FOR PRODUCING PHOTOGRAPHIC  
FILM HAVING A MAGNETIZABLE LAYER  
THEREON AND SUCH A PHOTOGRAPHIC FILM**

**BACKGROUND OF THE INVENTION**

**1. FIELD OF THE INVENTION**

The present invention relates to a process for producing photographic film having a magnetizable layer thereon and to such a film. More particularly, it relates to a process for providing on a movie film a sound track composed of a magnetic substance and to such a movie film.

**2. DESCRIPTION OF THE PRIOR ART**

As processes to provide a sound track on a movie film, there are two processes: one being an optical process and the other using a magnetic substance. The present invention belongs to the latter class.

Heretofore, a magnetizable layer has been applied to a movie film by applying a dispersion of a magnetizable substance to a development-processed movie film. However, this process has the defect that since images are first recorded and then sound is recorded, images and sound cannot be recorded at the same time. Therefore, with movie film having previously provided thereon a magnetizable layer it has been desired to remove the above-described defect, i.e., to enable one to record both images and sound at the same time.

On the other hand, in general, an antihalation layer is provided as a backing layer on a movie film, which antihalation layer can be removed with ease in the alkali development processing of the film.

In order to provide a magnetizable layer on a light-sensitive movie film, it is necessary to apply a dispersion of a magnetic substance onto the alkali-soluble antihalation layer provided as a backing layer. However, even when a normally employed dispersion of a magnetic substance is applied per se to the antihalation layer, the magnetizable layer formed is easily removed in the alkali development processing.

**SUMMARY OF THE INVENTION**

The present invention relates to a process for strongly adhering a magnetizable layer to an antihalation layer on a movie film, where the antihalation layer at the portion on which the magnetizable layer has been coated is rendered insoluble in the alkali development processing used for such movie films, and to movie films thus produced.

According to the present invention, it has been found that in provided a magnetizable layer on a light-sensitive movie film, the magnetizable layer can be strongly adhered to the antihalation layer to the extent that the magnetizable layer is not removed in the development processing by applying a dispersion of a magnetic substance onto the antihalation layer after adding to the dispersion a compound having at least 2 isocyanato groups or thioisocyanato groups, or by previously processing the portion of the antihalation layer where the magnetizable layer is to be coated with a solution containing such a compound.

**DETAILED DESCRIPTION OF THE INVENTION**

Preferred compounds within this class have from 2 to 4 isocyanato groups or thioisocyanato groups. This is because at the present time it is difficult to commercially obtain compounds having more than 4 isocyanato groups or thioisocyanato groups at reasonable cost.

As the binder for the antihalation layer, there are preferably used alkali soluble resins such as cellulose esters of dicarboxylic acids or vinyl copolymers containing maleic anhydride. Examples of cellulose esters of dicarboxylic acids are cellulose acetate phthalate, cellulose acetate maleate, hydroxalkyl alkyl cellulose tetrahydrophthalate, hydroxalkyl alkyl cellulose hexahydrophthalate (alkyl moiety thereof having from 1 to 4 carbon atoms and including a methyl, ethyl, propyl or butyl), and the like. Examples of vinyl copolymers containing maleic anhydride are maleic anhydride-styrene copolymers, maleic anhydride-styrene derivative copolymers, maleic anhydride-alkyl acrylate copolymers, maleic anhydride-alkyl methacrylate copolymers (alkyl moiety thereof having from 1 to 4 carbon atoms and including a methyl, ethyl, propyl and butyl groups), and the like. Examples of styrene derivatives include methylstyrene and p-chlorostyrene.

The dispersion for use in forming the antihalation layer suitable comprises 0.1 - 2% by weight of a mixture of carbon black and the above described binder (mixing ratio: 10 parts by weight : 15 - 50 parts by weight), balance organic solvent. The average particle size of the carbon black is preferably 20 - 30  $\mu$ .

In particular, the present invention is especially effective in the case wherein there is used, as the binder for the antihalation layer, a copolymer of maleic anhydride and styrene, a styrene derivative, an alkyl acrylate (alkyl moiety having 1 - 4 carbon atoms), an alkyl methacrylate (alkyl moiety having 1 - 4 carbon atoms) or the like, cellulose acetate phthalate, cellulose acetate maleate, hydroxalkyl alkyl cellulose tetrahydrophthalate (alkyl moiety having 1 - 4 carbon atoms), hydroxylalkyl alkyl hexahydrophthalate (alkyl moiety having 1 - 4 carbon atoms), etc., with the copolymerization ratio of the vinyl copolymer containing maleic anhydride being 1:1, and preferred styrene derivatives including, for example, methylstyrene, p-chlorostyrene, etc.

An antihalation layer to be provided on the surface of a photographic film opposite to the surface on which a light-sensitive silver halide emulsion layer is coated is designed to be alkali soluble. The antihalation layer is provided in order to prevent diffused reflection of incident rays upon photographing. The antihalation layer is designed so that it will be dissolved and removed in the step of photographic processing, particularly, development processing (the developer being alkaline). After such treatment, the film becomes transparent.

Therefore, if a magnetic recording layer is merely provided on the antihalation layer, the magnetic recording layer will be separated from the photographic film due to the removal of the antihalation layer bonding both layers. For this reason, the antihalation layer is rendered alkali insoluble by adding a compound or compounds containing isocyanato groups or thioisocyanato groups to the magnetic recording layer, or, by processing before coating the magnetic recording layer, only the portion of the antihalation layer on which the magnetic recording layer is to be coated is rendered alkali insoluble.

The reason why the antihalation layer is made insoluble in the alkali development processing by applying a dispersion of a magnetic substance after adding thereto a compound having two or more isocyanato groups or thioisocyanato groups, or by processing the portion of the antihalation layer on which portion the magnetiz-

able layer is to be provided with a solution containing a compound having one or more isocyanato groups or thioisocyanato groups, is considered to be that the applied compound diffuses into the antihalation layer and reacts with carboxyl groups present in the binder to form a two dimensional or three dimensional network structure in the binder. In general, the carboxyl groups are not in a salt form while contained in the antihalation layer, and are converted to a  $-\text{COOM}$  (M : alkali) type salt in alkali solution (i.e., upon development processing). As a result of this reaction, the antihalation layer becomes alkali soluble and is delaminated from the film. Therefore, carboxyl groups are not in a salt form before treating with an alkali solution.

Typical examples of the compound (or compounds, since mixtures can be used) used in the invention having at least 2 isocyanato groups or thioisocyanato groups are illustrated below.

Compound (I)  $\text{OCN}(\text{CH}_2)_n\text{NCO}$  n=2-12,

Compound (II)  $\text{OCN}(\text{CH}_2)_m-\text{X}-(\text{CH}_2)_n\text{NCO}$  X=O or S,  
m, n=2-4,

Compound (III)  $\text{SCN}(\text{CH}_2)_n\text{NCS}$  n=2-10,

Compound (IV)  $\text{OCNCH}_2-\text{C}(\text{CH}_3)_2-\text{CH}_2-\text{CH}(\text{CH}_3)\text{CH}_2\text{CH}_2\text{NCO},$

Compound (V) 

Compound (VI) 

wherein the floating NCX group is located at the 0—, m— or p-position to R, X represents O or S, and R represents a hydrogen atom or a methyl group,

Compound (VII) 

where  $n$  is 0 or 1,

Compound (VIII) 

wherein Y represents a hydrogen atom or NCO, and R1 represents a hydrogen atom or



Compound (IX)



Compound (X)



15

wherein  $R_2$  represents a  $C_1 - C_6$  alkyl group, and Compound (XI)



20

The amount of the compound (or compounds, since mixture can be used) having isocyanato groups or thioisocyanato groups to the dispersion of magnetic substance varies depending upon the kind of the compound, kind of the solvent for the dispersion, etc., i.e., compounds having a larger molecular weight are added in a greater amount, and compounds having less  $-\text{NCX}$  groups in number are added in a greater amount (molar numbers). Further, the permeation speed of the solvent into the antihalation layer varies depending upon the combination of the binder used in the antihalation layer and the solvent. Where a solvent having a faster penetration speed is employed, the amount may be less since the isocyanato or thioisocyanato compound penetrates rapidly together with the solvent. However, the compound is preferably added to the dispersion of magnetic substance in an amount of 0.05% to 7% by weight, based on the total weight of the magnetic dispersion (% by weight).

Further, in the case of processing the antihalation layer prior to providing the magnetizable layer, it is desirable to conduct the processing with a solution containing 0.05% - 10% (by weight) of the compound, based on the total weight of the coating solution (% by weight). Most preferably, the dried thickness of the magnetic layer is about 7 to about 13 microns. The amount of compound in  $\text{g}/\text{cm}^2$  can be calculated from both the amount added to the magnetic dispersion and the thickness described above.

Where the antihalation layer is processed with a solution containing isocyanato or thioisocyanato compound, the dried thickness of this processing solution is  $1/10 - 1/50$  the dried thickness of the magnetic recording layer. When a separate solution of the compound is used, it is preferably applied in a binder. The binders are suitably those exemplified above for the magnetic recording layer, and the binder can be used in amounts as recited from the magnetic recording layer, e.g., on the order of about 5 to about 20 wt.% of the solvent, the solution containing the compound(s) in an amount as recited above.

The separate solution can be applied over or under the antihalation layer, and can be in a layer which serves a dual function, e.g., as a subbing layer, where the amount of the compound is as defined above.

As the dispersion of a magnetic substance, those generally used for providing a sound track on a development-processed movie film for cinema can be employed. The coating solution for forming magnetic recording layer generally contains a ferromagnetic powder(s), binder and solvent.

The composition can be described as follows:

|                         |                                                        |
|-------------------------|--------------------------------------------------------|
| ferromagnetic powder(s) | about 15 to about 45 wt.%,<br>preferably 20 - 40 wt.%, |
| binder                  | about 5 to about 20 wt.%,<br>preferably 7 - 20 wt.%,   |
| solvent                 | about 35 to about 80 wt.%,<br>preferably 40 - 73 wt.%, |

The ferromagnetic powder can be  $\gamma$ - $Fe_2O_3$ ,  $\gamma$ - $Fe_2O_3$  containing Co,  $Fe_3O_4$ ,  $Fe_3O_4$  containing Co,  $CrO_2$ , CO-Ni-Fe alloys or mixtures thereof, e.g., as described in Japanese Pat. Nos. 14090/69; 18372/70; 22062/72; 22513/72; 28466/71; 38755/71; 4286/72; 12422/72; 17284/72; 18509/72; 18573/72; and the like.

As the binder used for the recording layer in the present invention, a conventionally known thermoplastic resin, thermosetting resin, (or reaction-type resin) or mixtures thereof are used.

As the thermoplastic resins, those having a softening point of less than 150°C, a mean molecular weight of about 10,000 to about 200,000 and a copolymerization degree of about 400 to about 500, such as vinyl chloride-vinyl acetate copolymers, vinyl chloride-vinylidene chloride copolymers, vinyl chloride-acrylonitrile copolymers, acrylate-acrylonitrile copolymers, acrylate-vinylidene chloride copolymers, acrylate-styrene copolymers, methacrylate-acrylonitrile copolymers, methacrylate-vinylidene chloride copolymers, methacrylate-styrene copolymers, urethane elastomers, nylon-silicone resins, nitrocellulose-polyamide resins, polyvinyl fluorides, vinylidene chloride-acrylonitrile copolymers, butadiene-acrylonitrile copolymers, polyamide resins, polyvinyl butyrals, cellulose derivatives, styrene-butadiene copolymers, polyester resins, chlorovinyl ether-acrylate copolymers, amino resins, various synthetic rubber thermoplastic resins, and the like, are used.

Specific examples of such resins are illustrated in Japanese Pat. Nos. 6877/62; 12528/64; 19282/64; 5349/65; 20907/65; 9463/66; 14059/66; 16985/66; 6428/67; 11621/67; 4623/68; 15206/68; 2889/69; 17947/69; 18232/69; 14020/70; 14500/70; 18573/72; 22063/72; 22064/72; 22068/72; 22069/72; 22070/72; 27886/72; and the like.

The thermosetting resin or reaction-type resin used preferably has a molecular weight of less than about 200,000 in the state of a coating solution and, upon heating after coating and drying, the molecular weight becomes infinite due to the reaction of condensation, addition etc. Of these resins, those which are not softened or melted before the thermal condensation are preferred. To be specific, there are, for example, phenol resins, epoxy resins, polyurethane thermosetting-type resins, urea resins, melamine resins, alkyd resins, silicone resins, acrylic reactive resins, epoxy-polyamide

resins, nitrocellulosemelamine resins, a mixture of a high molecular weight polyester resin and an isocyanate prepolymer, a mixture of a methacrylate copolymer and a diisocyanate prepolymer, a mixture of polyester polyol and a polyisocyanate, urea-formaldehyde resins, a mixture of a low molecular weight glycol/high molecular weight diol/triphenylmethane-isocyanate, polyamide resins and mixtures thereof.

Such resins are illustrated in Japanese Pat. Nos. 10 8103/64; 9779/65; 7192/66; 8016/66; 14275/66; 18179/67; 12081/68; 28023/69; 14501/70; 24902/70; 13103/71; 22065/72; 22066/72; 22067/72; 22072/72; 22073/72; 28045/72; 28048/72; 28922/72; and the like.

15 The magnetic recording layer is formed by dissolving the above-described composition in an organic solvent and applying the resulting coating solution to the antihalation layer. As the organic solvent used upon coating, there can be employed ketones such as acetone,

20 methyl ethyl ketone, methyl isobutyl ketone, cyclohexanone, etc., alcohols such as methanol, ethanol, propanol, butanol, etc.; esters such as methyl acetate, ethyl acetate, butyl acetate, propyl acetate, amyl acetate, ethyl lactate, glycol acetate, monoethyl ether, etc.; ether; glycol ethers such as glycol dimethyl ether, glycol monoethyl ether, dioxane, etc.; aromatic hydrocarbons such as benzene, toluene, xylene, etc.; chlorinated hydrocarbons such as methylene chloride, ethylene chloride, carbon tetrachloride, chloroform, trichloroethane, ethylene chlorhydrin, dichlorobenzene, and the like.

Any of the solvents used to form the magnetic layer can also be used as solvents in the case where the compound having at least two isocyanato or thioscyanato groups is directly applied to the antihalation layer. As the preferred solvents used, there are ketones, e.g., acetone, methyl ethyl ketone, cyclohexanone, etc., esters, e.g., methyl acetate, ethyl acetate, propyl acetate, butyl acetate, amyl acetate, etc., chlorinated hydrocarbons, e.g., methylene chloride, ethylene chloride, trichloroethane, etc., dioxane, tetrahydrofuran, morpholine, dimethylformamide, methyl cellosolve acetate, aromatic hydrocarbon such as benzene, toluene and xylene and the like, used alone or in suitable combinations.

45 The solvent used can vary depending upon the binder for the dispersion of the magnetic recording layer, the binder for the antihalation layer and the isocyanato or thioscyanato compounds. However, a proper solvent can be selected with ease by a person skilled in the art the following points in mind:

1. the solvent should dissolve the binder for the magnetic recording layer;
2. the solvent should dissolve the isocyanato or thioscyanato compound;
3. the solvent should dissolve or swell the binder for antihalation layer; and
4. the solvent should not react with the compounds or components described in the above articles (1) - (3).

60 In addition, the solvent should be selected considering a boiling point, etc., suitable for the coating or drying process.

65 The present invention will now be illustrated in more detail by several non-limiting examples of preferred embodiments of the invention. Solution compositions in the example are expressed in terms of parts by weight.

All movie film in the Examples comprised standard gelatino silver halide light sensitive emulsions for use in color photography coated on the side of the support opposite the antihalation layer and magnetic recording layer.

## EXAMPLE 1

A mixture of a polycondensation ester (between terephthalic acid and both ethylene glycol and triethylene glycol) and cellulose ester was applied to a polyethylene terephthalate support which had been crystallized by biaxial stretching, to form a subbing layer, on which a solution having the following composition was applied and dried at 100°C for 10 minutes to form an antihalation layer.

|                                                                  |    |
|------------------------------------------------------------------|----|
| Copolymer between styrene and maleic anhydride (1:1 molar ratio) | 10 |
| Carbon black (20 - 30 m $\mu$ particle size)                     | 5  |
| Methanol                                                         | 40 |
| Acetone                                                          | 60 |

The polycondensation ester had the following composition. A polyester was formed by adding an ester exchange reaction catalyst to a mixture of 1 mol. of dimethyl terephthalate, 1.7 moles of ethylene glycol, and 0.8 mol of triethylene glycol.

The cellulose ester was cellulose triacetate. The mixture for subbing layer has the following composition. Into a mixed solvent of 52 parts of ethylene dichloride, 8 parts of methylene chloride, 20 parts of methanol, 20 parts of tetrachloroethane and 20 parts of phenol were dissolved 0.2 part of the above-prepared polyester and 0.2 part of the cellulose triacetate, and the coating solution was applied to the surface of the polyethylene terephthalate film at 80°C. and dried for 6 minutes at 100°C. The procedure is in accordance with Example 1 of U.S. Pat. No. 3,492,122.

To the antihalation layer thus formed on the light-sensitive movie film for use in color photography there was applied a dispersion of a magnetic substance having the following composition which was then dried at 40°C for 3 minutes.

|                                                                                                                      |     |
|----------------------------------------------------------------------------------------------------------------------|-----|
| Nitrocellulose (M.W. ca 70,000-80,000)                                                                               | 10  |
| Ferromagnetic $\gamma$ -Fe <sub>2</sub> O <sub>3</sub> (average particle size: 0.8 $\times$ 0.1 $\times$ 0.1 micron) | 30  |
| Diethyl phthalate                                                                                                    | 2   |
| Ethyl acetate                                                                                                        | 20  |
| Butyl acetate                                                                                                        | 30  |
| Cellosolve acetate                                                                                                   | 10  |
| Compound (IV)                                                                                                        | 0.5 |

When the resulting movie film having thereon the resulting magnetizable layer (ca 8-10 $\mu$  thick) was subjected to standard color development processing, i.e., first development, stopping, hardening, color development, stopping, hardening, washing with water, bleaching, washing with water, fixing, washing with water, stabilization and drying, the magnetizable layer was not delaminated but strongly adhered to the support. On the other hand, in the case of not adding compound (IV), the magnetic layer was removed during the development processing.

## EXAMPLE 2

A solution having the following composition was applied to the antihalation layer of a light-sensitive movie film as in Example 1 having the same antihalation layer as in Example 1, and dried at 40°C for 3 minutes.

|    |                                        |    |
|----|----------------------------------------|----|
| 10 | Nitrocellulose (M.W. ca 60,000-80,000) | 2  |
|    | Acetone                                | 40 |
|    | Butyl acetate                          | 30 |
|    | Dioxane                                | 30 |

## Compound (V)

Subsequently, a dispersion of a magnetic substance having the following composition was applied thereto and dried at 50°C for 3 minutes. Too high a temperature or too long a drying time exerts a detrimental influence on the photographic emulsion layer and is therefore not favorable. Preferable ranges are about 30° - 60°C in temperature and about 2 - 20 minutes in drying time.

|    |                                                                                  |    |
|----|----------------------------------------------------------------------------------|----|
| 25 | Vinyl chloride/vinyl acetate copolymer (85:15, mol %)                            | 5  |
|    | epoxy resin                                                                      | 5  |
|    | Nitrile rubber having low polymerization degree (acrylonitrile-butadiene rubber) | 2  |
| 30 | Methyl ethyl ketone                                                              | 30 |
|    | Toluene                                                                          | 30 |
|    | Iron oxide (same as in Example 1)                                                | 30 |

35 When the thus obtained film having thereon the resulting magnetizable layer (ca 8 - 10 $\mu$  thick) was alkali-processed as in Example 1 and used in a projector equipped for magnetically recording and reproducing sound and projecting repeatedly 200 times, no damage 40 was observed in the magnetizable layer.

## EXAMPLE 3

An antihalation layer was formed on a light-sensitive movie film for color photography comprising a cellulose triacetate support by applying a solution having composition (A) and drying the same. Then, a dispersion of a magnetic substance containing different compounds having isocyanato groups or thioisocyanato groups as shown by composition (B) was applied and dried at 40°C for 3 minutes.

|    |                                                    |    |
|----|----------------------------------------------------|----|
| 55 | Composition (A)                                    |    |
|    | Hydroxymethyl methyl cellulose tetrahydrophthalate | 10 |
|    | Carbon black (20 - 30 m $\mu$ particle size)       | 5  |
|    | Acetone                                            | 70 |
|    | Methanol                                           | 30 |
| 60 | Composition (B)                                    |    |
|    | Nitrocellulose (MW ca 50,000 - 80,000)             | 10 |
|    | Iron oxide (same as in Example 1)                  | 30 |
|    | diethyl phthalate                                  | 2  |
|    | Isoamyl acetate                                    | 20 |
|    | Acetone                                            | 20 |
|    | Dioxane                                            | 20 |

65 The results obtained by subjecting the resulting films to alkali development processing as in Example 1 were as follows.

| Compound                                                         | Amount added | Alkali development processing                                         |
|------------------------------------------------------------------|--------------|-----------------------------------------------------------------------|
| 1 Compound (I), n=6                                              | 0.4          | Strongly adhered even after development processing.                   |
| 2 Compound (II), n=6                                             | 0.5          | do.                                                                   |
| 3 Compound (IV)                                                  | 0.6          | do.                                                                   |
| 4 Compound (V)                                                   | 0.8          | do.                                                                   |
| 5 Compound (X),<br>R <sub>2</sub> =C <sub>2</sub> H <sub>5</sub> | 1.0          | do.                                                                   |
| 6 —                                                              | 0            | The magnetizable layer was delaminated during development processing. |

While the invention has been described in detail and with reference to specific embodiments thereof, it will be apparent to one skilled in the art that various changes and modifications can be made therein without departing from the spirit and scope thereof.

What is claimed is:

1. A process for producing a photographic film having thereon a magnetic recording layer by applying a dispersion of a magnetic substance to an antihalation layer of a light-sensitive film for cinema, wherein the dispersion contains a compound or compounds, having at least two isocyanato groups or thioisocyanato groups capable of rendering said antihalation layer alkali insoluble, thereby rendering said antihalation layer alkali insoluble.

2. The process as claimed in claim 1 wherein said dispersion of magnetic substance comprises from about 15 to about 45% by weight of ferromagnetic powder, from about 5 to about 20% by weight of binder, and from about 35 to about 80% by weight of solvent.

3. The process as claimed in claim 2 wherein said dispersion contains 0.05 to 7% by weight, based on said dispersion, of said compound.

4. The process as claimed in claim 1 wherein said compound has from 2 to 4 isocyanato groups or thioisocyanato groups.

5. The process as claimed in claim 4 wherein said compound is selected from the group consisting of Compounds (I) to (XI) below:

|                |                                                                                                             |                        |
|----------------|-------------------------------------------------------------------------------------------------------------|------------------------|
| Compound (I)   | OCN(CH <sub>2</sub> ) <sub>n</sub> NCO                                                                      | n=2-12,                |
| Compound (II)  | OCN(CH <sub>2</sub> ) <sub>m</sub> -X-(CH <sub>2</sub> ) <sub>n</sub> NCO                                   | X=O or S,<br>m, n=2-4, |
| Compound (III) | SCN(CH <sub>2</sub> ) <sub>n</sub> NCS                                                                      | n=2-10,                |
| Compound (IV)  | OCNCH <sub>2</sub> -C(CH <sub>3</sub> ) <sub>2</sub> -CH <sub>2</sub> -CH <sub>2</sub> CH <sub>2</sub> NCO, |                        |
| Compound (V)   |                                                                                                             |                        |
| Compound (VI)  |                                                                                                             |                        |

wherein the floating NCX group is located at the o-, m-, or p-position to R, X represents O or S, and R represents a hydrogen atom or a methyl group,

Compound (VII)



wherein n is 0 or 1,



wherein Y represents a hydrogen atom or NCO, and R<sub>1</sub> represents a hydrogen atom or



Compound (IX)



Compound (X)



35 wherein R<sub>2</sub> represents a C<sub>1</sub> - C<sub>6</sub> alkyl group, and



6. The process as claimed in claim 1 wherein said magnetic recording layer has from about 7 to about 13 microns of a dried thickness.

7. The process as claimed in claim 1 wherein said solution contains from 0.05 to 10% by weight, based on total weight of said solution, of said compound.

50 8. The process as claimed in claim 7 wherein the dried thickness of said processing solution is from about one-tenth to about one-fiftieth of the dried thickness of said magnetic recording layer.

9. A motion picture film having a magnetic recording 55 layer coated on the antihalation layer coating on the film support at the opposite side of the light sensitive photographic layer, said magnetic recording layer comprising a compound having at least two or more isocyanato groups or thioisocyanato groups capable of and thereby rendering said antihalation layer alkali insoluble.

10. The motion picture film as claimed in claim 9 wherein said magnetic recording layer is coated from a dispersion of the magnetic substance, which comprises from about 15 to about 45% by weight of ferromagnetic powder, from about 5 to about 20% by weight of binder, and from about 35 to about 80% by weight of solvent.

11. The motion picture film as claimed in claim 10 wherein said dispersion contains from 0.05 to 7% by weight, based on said dispersion, of said compound.

12. The motion picture film as claimed in claim 9 wherein said compound has from 2 to 4 isocyanato groups or thioisocyanato groups.

13. The motion picture film as claimed in claim 12 wherein said compound is selected from the groups consisting of Compounds (I) to (XI) below:

Compound (I)  $OCN(CH_2)_nNCO$   $n=2-12$

Compound (II)  $OCN(CH_2)_m-X-(CH_2)_nNCO$   $X=O$  or  $S$ ,  $m, n=2-4$

Compound (III)  $SCN(CH_2)_nNCS$   $n=2-10$

Compound (IV)  $OCNCH_2-C(CH_3)_2-CH_2-CH-CH_2CH_2NCO$

Compound (V) 

Compound (VI) 

wherein the floating NCX group is located at the o-, m- or p-position to R, X represents O or S, and R represents a hydrogen atom or a methyl group,

Compound (VII) 

where  $n$  is 0 or 1,

Compound (VIII) 

wherein Y represents a hydrogen atom or NCO, and  $R_1$  represents a hydrogen atom or

Compound (IX) 

Compound (X) 

wherein  $R_2$  represents a  $C_1 - C_6$  alkyl groups, and



14. A motion picture film having a magnetic recording layer, a subbing layer, and an antihalation layer coated on the film support on the opposite side of the light sensitive photographic layer, said subbing layer comprising a compound having at least two or more isocyanato groups or thioisocyanato groups capable of rendering said antihalation layer alkali insoluble and being in contact with said antihalation layer, thereby rendering said antihalation layer alkali insoluble.

15. A motion picture film claimed in claim 14 wherein said compound has from 2 to 4 isocyanato groups or thioisocyanato groups.

16. A motion picture film claimed in claim 15 wherein said compound is selected from the group consisting of Compounds (I) to (XI) below:

Compound (I)  $OCN(CH_2)_nNCO$   $n=2-12$

Compound (II)  $OCN(CH_2)_m-X-(CH_2)_nNCO$   $X=O$  or  $S$ ,  $m, n=2-4$

Compound (III)  $SCN(CH_2)_nNCS$   $n=2-10$

Compound (IV)  $OCNCH_2-C(CH_3)_2-CH_2-CH-CH_2CH_2NCO$

Compound (V) 

Compound (VI) 

wherein the floating NCX group is located at the o-, m- or p-position to R, X represents O or S, and R represents a hydrogen atom or a methyl group,

Compound (VII) 

where  $n$  is 0 or 1,

Compound (VIII) 

wherein Y represents a hydrogen atom or NCO, and  $R_1$  represents a hydrogen atom or



13

Compound (IX)



Compound (X)



wherein  $R_2$  represents a  $C_1 - C_6$  alkyl group, and

Compound (XI)



17. A process for producing a photographic film having thereon a magnetic recording layer by applying a dispersion of a magnetic substance to an antihalation layer of a light-sensitive film for cinema, wherein the antihalation layer is processed with a solution containing a compound or compounds having at least two isocyanato groups or thioisocyanato groups capable of rendering said antihalation layer alkali insoluble before application of said dispersion, thereby rendering said antihalation layer alkali insoluble.

18. The process as claimed in claim 17 wherein said dispersion of magnetic substance comprises from about 15 to about 45% by weight of ferromagnetic powder, from about 5 to about 20% by weight of binder, and from about 35 to about 80% by weight of solvent.

19. The process as claimed in claim 17 wherein said compound has from 2 to 4 isocyanato groups or thioisocyanato groups.

20. The process as claimed in claim 19 wherein said compound is selected from the group consisting of Compounds (I) to (XI) below:

Compound (I)  $OCN(CH_2)_nNCO$  $n=2-12$ ,Compound (II)  $OCN(CH_2)_m-X-(CH_2)_nNCO$  $X=O$  or  $S$ ,  
 $m, n=2-4$ ,Compound (III)  $SCN(CH_2)_nNCS$  $n=2-10$ ,Compound (IV)  $OCNCH_2-C(CH_3)-CH_2-CH-CH_2CH_2NCO$ ,Compound (V)  $CH_3$   


14

Compound (VI)



5 wherein the floating  $NCX$  group is located at the o-, m-, or p-position to  $R$ ,  $X$  represents  $O$  or  $S$ , and  $R$  represents a hydrogen atom or a methyl group,

Compound (VII)



10

 $n=0$  or  $1$ ,

Compound



20

wherein  $Y$  represents a hydrogen atom or  $NCO$ , and  $R_1$  represents a hydrogen atom or



Compound (IX)



35

Compound (X)



40

wherein  $R_2$  represents a  $C_1 - C_6$  alkyl group, and

Compound (XI)



50

21. The process as claimed in claim 17 wherein said magnetic recording layer has a thickness of from about 7 to about 13 microns of a dried thickness.

\* \* \* \* \*

55

UNITED STATES PATENT OFFICE  
CERTIFICATE OF CORRECTION

PATENT NO. : 3,870,525  
DATED : March 11, 1975  
INVENTOR(S) : Nobuo YAMAMOTO et al

It is certified that error appears in the above-identified patent and that said Letters Patent are hereby corrected as shown below:

IN THE HEADING:

Foreign Application Priority Data

Delete "Apr. 12, 1972" insert --Apr. 24, 1972 --

Signed and sealed this 20th day of May 1975.

(SEAL)

Attest:

RUTH C. MASON  
Attesting Officer

C. MARSHALL DANN  
Commissioner of Patents  
and Trademarks